

Dec. 11, 1956

M. H. GOLDSCHEIN  
INSTANT DRYING PHOTOSTAT

2,773,769

Filed Jan. 29, 1953

*Fig. 1.*



*Fig. 2.*



*Fig. 3.*



*Fig. 4.*



INVENTOR

MAX H. GOLDSCHEIN  
BY  
H. L. Sodfrey  
ATTORNEY

## 1

2,773,769

## INSTANT DRYING PHOTOSTAT

Max H. Goldschein, Washington, D. C.

Application January 29, 1953, Serial No. 334,107

1 Claim. (Cl. 96—84)

(Granted under Title 35, U. S. Code (1952), sec. 266)

The invention described herein may be manufactured and used by or for the Government of the United States for governmental purposes without the payment to me of any royalty thereon in accordance with the provisions of the act of April 30, 1928 (Ch. 460, 45 Stat. L. 467).

This invention relates to photographic materials and, more particularly, to light sensitive elements for use in rapidly copying documents, drawings, and the like, under conditions present in the usual office.

The photographic elements used in commercial or large scale copying or reproducing establishments generally consists of sheets of white paper coated with a suitable light sensitive material, such as silver halide emulsion. This paper is stored under conditions preventing its exposure to actinic rays, and after its exposure in the printing operation, it must be carefully protected from further exposure during subsequent handling in developing and fixing operations. Since the paper is porous, it absorbs liquid and becomes thoroughly wet during development and washing. Dark rooms and expensive handling and drying equipment are necessary in photographic reproduction with this type of material. The operations are also time consuming.

It is frequently desirable to make a photographic copy of a document, drawing, or the like, for immediate use, under conditions where it is inconvenient or impossible to remove the original to a photographic establishment provided with the customary bulky apparatus, dark rooms, and washing and drying equipment. Small offices may resort to the use of less complicated apparatus with improvised dark rooms, but this unduly disturbs the office routine and time is lost in drying the washed prints. The portable self-contained photocopying apparatus disclosed in my Patent No. 2,557,097 solves many of the problems encountered in small scale photographic reproduction work of the type described. However, when the usual photosensitive paper is used in this apparatus, a special covering sheet of tinted cellophane, or the like, must be used as a cover for daylight handling of the exposed print, and the final washed print must be squeezed and blotted free of the absorbed moisture. Unskilled operators may have difficulty in avoiding overexposure of the print during the handling thereof.

An object of this invention is to provide a light sensitive material for photocopying, of the type described, which may be handled under substantially daylight conditions and which after developing, fixing and washing may be quickly dried for immediate use.

Another object of this invention is to provide a light sensitive material for photocopying which is substantially hydrophobic and which is protected on one side from the passage of actinic rays.

Another object of this invention is to provide photographic sheet materials of water resistant plastic coated or impregnated to provide a white background and provided on one side with a red-tinted layer and on the opposite side with a light sensitive emulsion.

## 2

These and other objects and advantages of the invention will become apparent from the following description, and from the drawings, in which:

Fig. 1 is an enlarged, diagrammatic, fragmentary, sectional view of light sensitive plastic sheet materials illustrating one embodiment of the invention.

Fig. 2 is a view similar to that of Fig. 1 of light sensitive sheet material illustrating another form of the invention.

Fig. 3 is a view similar to that of Fig. 1 of light sensitive sheet material illustrating another form of the invention.

Fig. 4 is a view similar to that of Fig. 1 of light sensitive sheet material illustrating still another form of the invention.

The photographic material of this invention comprises, in general, a translucent or semi-opaque, water-resistant sheet, one side of which is sensitive to light and the other side of which is tinted to retard the passage of actinic rays.

The photographic sheet materials are made up of a flexible support of white, substantially hydrophobic, or water-resistant plastic material, or of a hydrophobic plastic material pigmented or coated with a suitable substance to provide a white background having a coating of light sensitive emulsion on one side, and having a red tint on the opposite side of the sheet from the light sensitive material to retard the passage of light rays. The tinted surface may be in the form of a separate water-resistant, water soluble, or strippable plastic coating, or may comprise a permanent part of the plastic support as hereinafter specified.

Suitable water-resistant support materials comprise plastic sheet or film material fabricated from polyvinyl chloride, polythene, vinylidene chloride polymers and copolymers known to the art as Saran, polystyrene, methyl methacrylate polymer, and the like. Regenerated cellulose, such as cellophane, which has been rendered moisture resistant during the process of manufacture may also be used as support materials. For example, Saran-coated cellophane, which is high resistant to moisture, may be employed. Cellulose acetate and other plastics that normally absorb moisture, or possess low water resistance, may likewise be waterproofed by suitable surface coatings or by other means applied during the process of manufacture, and may subsequently be utilized as support materials in accordance with this invention. Suitable support material may also comprise paper made hydrophobic or water-resistant by incorporating a suitable water-resistant plastic or resin binder with said paper. For example, the paper may be impregnated with polystyrene, or it may be coated with methyl methacrylate polymer, or with vinylite resins. All of the above-mentioned materials are generally designated herein as water-resistant plastic sheet material. It will be understood that the plastic sheet materials should incorporate sufficient plasticizers to render them adequately flexible for rolling without cracking or breaking.

In order to provide a proper white background for photostatting, the plastic support material is pigmented during its process of manufacture or is coated with a suitable white pigment material after being formed into sheets. Metal oxides such as titanium dioxide, zinc oxide, and the like may be used as the pigment for impregnating or coating the plastic support. Sufficient white pigment is employed to render the sheet material translucent or substantially opaque. However, the resulting white sheet should permit the passage of actinic rays for reasons hereinafter apparent. Ordinary white paper which has been waterproofed by the methods described provides an adequate background.

Where the water-resistant plastic sheet material includes a white pigment whereby the proper background

is provided for printing, a separate coating of red-tinted material is applied to one side thereof, to retard the passage of actinic rays. This coating may comprise a plastic material similar to that of the support, but incorporating a suitable red dye in place of the white pigment. The coating may also comprise soluble materials such as gelatin which are suitably tinted. The red-tinted plastic may be incorporated in a suitable solvent and applied as a thin layer to one side of the white support material. Alternatively, a separate red-tinted plastic sheet may be cemented to the support sheet with a suitable plastic cement. This sheet may be attached in such a manner that it can be stripped from the support if desired. It will be understood that any red-tinted plastic material which is easily applied and sufficiently flexible may be used as the support coating.

A light sensitive emulsion, such as gelatin containing silver salts, is now applied to the side of the support opposite the tinted coating. Should difficulty be encountered with some of the water-resistant materials in securing adequate adhesion of the gelatin layer, a suitable substratum material may first be applied in the manner known to the art.

In a further embodiment of the invention, a red-tinted, water-resistant plastic sheet material is utilized as the support. This is coated with a suitable white pigment to form the background for printing. The light sensitive emulsion is then applied over the pigment layer.

Referring now to the drawings for a more detailed description of the invention, Fig. 1 shows a white, water-resistant, plastic support, such as polyvinyl chloride containing a small amount of titanium dioxide, having a coating 11 on one side thereof of red-tinted material such as polyvinyl chloride or of gelatin tinted with a suitable red dye. The material forming the coating 11 may be dissolved or stripped off during developing operations if desired. The other side of the support 10 from the tinted layer 11 is provided with a coating of silver halide gelatin emulsion 12.

In the embodiment of the invention shown in Fig. 2 of the drawings, a red-tinted, water-resistant plastic sheet forms a support 14. This support is coated with a suitable plastic coating agent containing a small amount of white pigment to form layer 15. The gelatin silver-halide emulsion is applied over the white pigment layer 15 to form a second layer 16.

In a third embodiment of the invention, as illustrated in Fig. 3, a white water-resistant support 17 comprises paper which has been impregnated with polystyrene. This support is coated on one side with red-tinted polyvinyl chloride, gelatin, or the like, to form layer 18. The silver-halide emulsion forms a layer 19 on the opposite side from the tinted coating as in the embodiment described in Fig. 1.

Fig. 4 shows a white paper 20 utilized as a support coated on one side with a thin coating of transparent polyvinyl chloride and on the other side with a red-tinted polyvinyl chloride layer 22. The paper 20 is rendered water-resistant by the coating materials, and one of the coating layers serves to retard the passage of actinic rays. The tinted layer 22 in this instance must be water resistant. The gelatin, silver emulsion is applied on the opposite side of the support 20 from the tinted coating 22 and over the transparent layer 21 to form light sensitive layer 23.

Each of the light sensitive sheet materials described above is highly water-resistant. The gelatin-silver halide emulsion is relatively thin and absorbs very little moisture during development, fixing and washing. The tinted coating is either water-resistant, as, for example, when polyvinyl chloride is used, or washes away in the developing bath as in the case of gelatin. After the washing operation, it is merely necessary to blot or sponge the print to remove droplets of water and the print is sufficiently dry for immediate use.

The photographic material described herein may be stored in the form of a roll, preferably with the red-tinted layer on the outer portion thereof to protect the light sensitive layer from exposure during handling. The material may be placed in any suitable device for exposure under a negative or under a document as the case may be. A suitable portable device for rapid photoprinting is described in my aforementioned Patent Number 2,557,097.

When a copy of a document is to be made and the document is printed on one side only, the light sensitive material is placed in the exposure device with the light sensitive emulsion side up. The document is placed face up on top of the light sensitive sheet. The material is then exposed for a suitable time to light passing through the document. Ordinary daylight may be used for making the exposure, or light from an incandescent lamp may be directed through the document to the light sensitive surface. After the proper exposure time, the document and sensitized sheet are removed from the exposure device and the sensitized sheet is quickly rolled up into a tight cylinder with the tinted layer outside. The roll of material may now be transported to the developing and fixing bath without further exposure. Where my portable device is used the developing, fixing, and washing liquids are contained in bottles and the roll of material is dipped first into the developing solution, then into the washing water, and then into the fixing solution and back into the wash water. The print is thereby developed, fixed and washed on the spot. It is now merely necessary to blot or sponge any adhering water from the print prior to its use. The water-resistant plastic material from which the print is made prevents absorption of moisture which would require the usual prolonged drying operations. The red-tinted outer layer retards the passage of actinic rays and prevents exposure prior to the development of the print. It will be understood that the procedure would be generally similar where means other than my portable apparatus are used for exposing, developing, fixing, and washing the print. However, greater care must be taken in most instances to avoid undue exposure of the print. In most operations, this can be avoided by keeping the red-tinted surface between the light and the light sensitive side of the sheet.

If the document to be copied is printed on both sides, the document is placed in an exposure device with the surface to be printed facing upward. The sheet material of this invention is then placed over the document with the sensitized side down. The exposure is made by directing light through the photosensitive sheet to the document. If the tinting is of a permanent type, the tinted surface retards the passage of actinic rays and a prolonged exposure must be made. Where the tinting is in the form of a strippable coating such coating is removed prior to the exposure. After the exposure is made, the print is developed as described above, the resulting print being a reverse or mirror image negative. The reverse negative is now placed over a new sheet of sensitized paper having its emulsion side up. The exposure and development are carried out as before and a positive print results. The time and equipment saved in drying the prints more than compensates for the extra time required in making the exposure even where the tinting is of a permanent type, and the prints may be more readily handled by amateurs without overexposure.

While the invention has been described with particular reference to the copying of documents, drawings, and the like, it will be understood that the materials described may be utilized for any purpose wherein a rapid-drying, light-protected printing roll is desired.

The photographic material shown above is by way of example only and many modifications will occur to those skilled in the art within the scope of the invention.

What is claimed is:

75 A rapid-drying, light-protected, non-projectible, com-

posite printing sheet comprising an opaque, water-imperious, flexible white sheet of polyvinyl chloride impregnated with zinc oxide, a light-sensitive silver halide coating on one surface of the sheet adapted to reproduce a latent image on exposure to light, the sheet carrying red tinting spaced from the light-sensitive coating resisting the passage of actinic rays through the sheet when rolled in storage, whereby further exposure of the latent image prior to development of the print is prevented, and the unrolled developed print immediately when drawn from 10 developing, fixing and washing baths is substantially in dry condition.

**References Cited in the file of this patent**

**UNITED STATES PATENTS**

1,597,727 De'Sperati ----- Aug. 31, 1926

1,631,421  
1,987,072  
2,199,580  
2,694,662

Lohofer ----- June 7, 1927  
McMaster ----- Jan. 8, 1935  
Tucker ----- May 7, 1940  
Hunter ----- Nov. 16, 1954

21,241  
114,933  
250,267  
303,752  
303,794  
316,811  
361,873  
509,316  
511,281

FOREIGN PATENTS  
Great Britain ----- of 1899  
Great Britain ----- Apr. 25, 1918  
Great Britain ----- July 1, 1927  
Great Britain ----- May 7, 1930  
Great Britain ----- May 8, 1930  
Great Britain ----- Aug. 8, 1929  
Great Britain ----- of 1931  
Great Britain ----- July 13, 1939  
Great Britain ----- Aug. 16, 1939